

## UNITED STATES PATENT OFFICE

EDWIN POTTER MENGEI, OF KNOXVILLE, TENNESSEE

## COLORING WALNUT VENEER SHEETS

No Drawing.

Application filed October 20, 1928. Serial No. 313,948.

This invention relates particularly to a method or process for coloring the sap wood of black walnut veneer sheets to make the color of the sap wood conform to or harmonize with the color of the heart wood.

It is known that the outer part of most black walnut logs is composed of a light or whitish wood called "sap wood", while the inner portion is of a dark or brownish gray 10 color and is called "heart wood". When the log is cut into veneer, the veneer produced from this whitish or sap portion has much less market value than has the veneer cut from the brownish gray or heart portion. For 15 example, sap walnut veneer 1/28 of an inch in thickness will sell for seven dollars per thousand feet, while the heart wood veneer of the same thickness and cut from the same log will bring approximately twenty dollars 20 per thousand feet. This difference in price is due to the fact that the brownish gray heart wood is much more desirable in the manufacture of furniture and similar work. Furniture manufacturers sometimes buy the 25 sap walnut veneer, glue it on panels or other bases, sand-paper it, and then color it superficially to resemble the heart wood veneer. But this process is unsatisfactory because of the extra labor involved and the deficient 30 coloring. That that method is unsatisfactory and substantially impractical is to be inferred from the fact that the manufacturers are willing to pay such difference in prices as I have above indicated.

The object of my invention is to impart 35 to the sap wood of the veneer sheet a coloring which will closely resemble the natural color of the heart wood.

A further object is to effect penetration 40 of such coloring of the sap wood part of a sheet of walnut veneer substantially uniformly through the sheet, and not limiting the coloring to the surfaces of the sheet. This is essential because the manufacturer, by 45 sanding, removes a part of the surface of the sheet after it has been glued to the piece of furniture or other base.

Another object of the invention is to perform the coloring without changing or damaging the fiber texture of the sheet, whereby

it would become difficult or impossible for the manufacturer to give the sheet surface a finish.

Another object of the invention is to effect the coloring of the sap wood part of such a sheet without materially changing the color or color shade of the heart wood of the same sheet. In this connection it is to be noted that some of the veneer sheets cut from the exterior of the log are all sap wood, while other sheets are composed in part of sap wood and in part of heart wood. In treating the sheets containing the light wood and the dark wood, the color of the dark wood is not to be materially changed.

My method or process of treating the veneer sheets is as follows:

Prepare a solution of hot water; chestnut extract (or tannic acid in any form) and a small percentage of iron salts ( $FeSO_4$  or  $FeCl_2$ ). I have obtained good results by measuring the chestnut extract and water of this solution in the proportion of one part of the extract to six parts of water. The solution is to be kept at less than the boiling point of water, preferably about  $160^{\circ}$  Fahrenheit. By experiment I have learned that, if the solution is kept at a temperature higher than above indicated, the tannic acid will break down and form other compounds which will produce a black scum on the surface of the veneer.

Then immerse the veneer sheets in this solution, and so arrange them that all portions will be reached by the solution. The sheets may be immersed when they are fresh from the cutting machine or after they have been dried.

After immersion has continued about eleven hours, the temperature of the solution having been maintained, the veneer is removed and placed in hot or boiling water to soften or dissolve or wash any objectionable deposits that may have formed on the surface of the sheets. If the tannic acid and the iron salts are fresh, and no objectionably high temperature has been reached in any part of the solution, such deposits will be absent and this washing step will not be necessary. Then, whether the washing step

has or has not been taken, the sheets are, preferably, rinsed in warm or hot water.

Next, the veneer sheets are removed and stacked upright so as to drain off as much of the solution as possible. The sheets are then dried in the usual manner of drying veneer sheets.

I have found, in practice, that the best procedure, in order to avoid checking, buckling, cracking, etc. of the sheets, is to allow the sheets to drain in an upright position for three or four hours.

Then partially dry the sheets in an ordinary mechanical hot-air drier at a temperature lower than ordinarily employed in such driers—preferably about 180° Fahrenheit. This drying is to be continued until the moisture content in the sheets is about nine per cent.

Then press the sheets flat in a hot plate drier to about a six per cent moisture content. This drying treatment seems to aid the coloring process and also to make the veneer sheets flat and tougher than would be expected after the immersion of the sheets in hot water.

In the practice of my invention, I make use of the fact that walnut wood contains some tannic acid or tannin. Tannic acid and iron salts ( $FeSO_4$  or  $FeCl_2$ ) have been used in making black ink. Through experimenting I found that, if a large quantity of tannic acid and a small quantity of iron salts are used, a brownish gray color (the color of walnut) is procured. If sap walnut veneer is immersed in a solution of iron salts and water, the iron acts on the tannin on the surface of the veneer, thus forming a black deposit, the surface of the veneer then being very dark while the inside remains light. The introduction of tannic acid in quantity hastens the process and prevents the objectionable black deposit and gives the desired brownish gray color throughout the wood.

But usually the "heart wood" contains a larger proportion of tanning or tannic acid than is contained in the "sap wood". Hence when the veneer sheets contain considerable parts of heart wood, the tannin delivered into the solution by the heart wood and the sap wood will be in sufficient quantity to render extraneous addition of tanning or tannic acid unnecessary.

When a veneer sheet is composed in part of "sap wood" and in part of "heart wood" and is subjected to the above method or process, the iron and tannic acid color the sap wood and seem to have little effect on the heart wood, so that it is generally impossible or difficult to tell where the sap wood and the heart wood meet. But even when the difference in coloring is sufficient to allow seeing the meeting line of the sap wood and the heart wood, that difference in coloring is so slight as to be unobjectionable in the trade.

In a solution kept at a temperature of approximately 170° Fahrenheit, the tannic extract remains in normal form approximately 100 hours. Thereafter the tannin is modified to such extent as to render the solution ineffective. But I have found that the normal or effective condition of the solution may be prolonged by acidifying it with a small quantity of acid such as sulphuric acid:

I claim as my invention:

1. In the art of coloring sap walnut veneer, the process which consists in immersing the veneer sheets in a solution of iron salts and tannic acid and water, in substantially the proportions stated, and keeping the solution at a temperature of approximately 160°, then removing the sheets and draining them; then partially drying the sheets; and then hot pressing the sheets.

2. In the art of coloring sap walnut veneer, the process which consists in immersing the veneer sheets in a solution of iron salts and tannic acid and water, in substantially the proportions stated, and keeping the solution at a temperature of approximately 160°, then removing the sheets and rinsing and draining them; then partially drying the sheets; and then hot pressing the sheets.

3. In the art of coloring sap walnut veneer, the herein described process which consists in exposing the veneer sheets to the action of a heated solution of water, tannic acid and iron salts, then draining, then partially drying; and then hot pressing the sheets.

4. In the art of coloring sap walnut veneer, the process which consists in exposing the veneer sheets to the action of a heated solution of water and iron salts, then rinsing, then partially drying; then hot pressing the sheets.

In testimony whereof I have signed my name, this sixteenth day of October, in the year one thousand nine hundred and twenty-eight.

EDWIN POTTER MENGEI.

110

115

120

125

130